

## UNITED STATES PATENT OFFICE

2,689,177

## CORROSION-RESISTANT ALLOY STEELS

George Henry Botham, Crawley, and John Frederick Lancaster and David Whitfield Outram Dawson, London, England, assignors to The A. P. V. Company Limited, London, England, a company of Great Britain

No Drawing. Application July 3, 1952,  
Serial No. 297,186

Claims priority, application Great Britain  
July 5, 1951

2 Claims. (Cl. 75—125)

1

This invention relates to corrosion resistant alloy steels, and particularly though not exclusively to stainless steels.

Alloy steels, the composition of which has been chosen to render them resistant to corrosion, are frequently very difficult to machine. Austenite-bearing stainless steels, in particular are always very difficult to machine. It is now common practice when such steels have to be machined to add to them in the melting shop small quantities of free cutting elements such as selenium, tellurium, phosphorus and sulphur but especially the latter. The addition of those elements, however, affects adversely to varying degrees the resistance of the steel to corrosion. For example a stainless steel containing 26% chromium, 4% nickel and 1% manganese may be rendered more liable to corrosion by the addition of 0.2% sulphur.

The decrease of corrosion resistance may be due to the formation of metallic compounds with the free cutting elements and in particular, when sulphur is the free cutting element used, manganese sulphide is formed if manganese is present in the alloy. Manganese sulphide is soluble in dilute acid media and gives rise to sulphuretted hydrogen. This gas is known to have a depassivating effect on stainless steel and may cause such alloys to become "active" in environments where they are normally passive, as shown in the following examples:

which most readily combines with the said free cutting element.

The selection of free cutting element will vary but the invention is of especial value when, as is most usual, the free cutting element added is sulphur. The metal included to combine with the sulphur must be more readily capable of combining with the sulphur than any other metal present in the alloy. Suitable metals may be selected by a consideration of known thermodynamical data but it may be observed that manganese and zirconium which very readily combine with sulphur to form acid soluble sulphides are inevitably excluded.

15 The alloys of this invention may therefore be arrived at by two routes. In one method the alloy may comprise those elements which alloy to provide the basic structure of the alloy, e. g. alloys of iron with chromium, nickel, molybdenum or vanadium or mixtures thereof, the said alloys being substantially free from any metal such as manganese or zirconium which would combine with the free cutting element more readily than the said alloying metals.

20 In the second method there may be added to an alloy a proportion of a metal which while not essential to the basic structure of the alloy nevertheless combines preferentially with the free cutting element.

25 One embodiment of the invention consists of a

30

| Composition |             |             |             |            | Machina-<br>bility | Solution rate (mgs.<br>loss per sq. deci-<br>metre per day)<br>in boiling 1%<br>Lactic Acid plus<br>1% NaCl |
|-------------|-------------|-------------|-------------|------------|--------------------|-------------------------------------------------------------------------------------------------------------|
| Cr, percent | Ni, percent | Mo, percent | Mn, percent | S, percent |                    |                                                                                                             |
| 18.1        | 7.8         | 2.5         | 1.1         | 0.34       | Free               | 118                                                                                                         |
| 18.5        | 8.0         | 2.6         | 1.1         | 0.04       | Difficult          | 16                                                                                                          |
| 18.3        | 7.6         | 0.05        | 1.0         | 0.34       | Free               | 1,340                                                                                                       |
| 18.3        | 7.9         | 0.05        | 1.1         | 0.03       | Difficult          | 890                                                                                                         |
| 21.7        | 5.2         | 1.6         | 1.0         | 0.28       | Free               | 490                                                                                                         |
| 22.3        | 4.8         | 1.6         | 0.9         | 0.03       | Difficult          | 46                                                                                                          |
| 26.8        | 4.4         | 0.05        | 1.0         | 0.29       | Free               | 6,200                                                                                                       |
| 26.3        | 4.9         | 0.3         | 0.9         | 0.01       | Difficult          | 285                                                                                                         |

It is a main object of the present invention to minimize the loss of resistance to corrosion of alloy steels, and in particular of stainless steels, to which have been added free cutting elements to render them readily machinable.

According to the present invention an alloy steel of easy machinability and high corrosion resistance comprises a free cutting element and includes within its composition a metal which combines with the said free cutting element to form an acid resistant compound or complex, said metal being, of those contained in the alloy, that

45 stainless steel rendered readily machinable by the addition of from 0.1% to 0.75% by weight of sulphur and not containing any metal, for example manganese or zirconium, such as will combine with said sulphur in preference to copper which forms an acid-insoluble sulphide, and wherein from 0.1% to 10% by weight of copper is added, the ratio of copper to sulphur being always in excess of 5:1.

50 In a particular embodiment of the invention a stainless steel contains by weight 26% chromium, 4% nickel, 0.2% sulphur and 2.5% copper, and

does not contain any substantial amount of any metal, for example manganese or zirconium, such as will combine with sulphur in the presence of copper.

The chemical tests carried out on a stainless steel to discover its resistance to corrosion often include immersion of the steel in nitric acid, and immersion in sodium chloride solution containing an organic acid such as lactic acid. Stainless steel containing 26% chromium, 4% nickel and 1% manganese (referred to above) gives satisfactory results in these tests, but with the addition of 0.2% sulphur to render it readily machinable it gives very poor results. It is believed that, at high temperatures, for instance about 1500° C., the sulphur combines with the manganese to form manganese sulphide which, dispersed in fine particles through the steel, promotes the breaking up of swarf in machining. The manganese sulphide is, however, soluble in dilute nitric and hydrochloric acids, and on going into solution causes corrosion of the steel. The hydrogen sulphide which is formed further acts as a depassivator.

The replacement, in the steel previously mentioned containing 26% chromium, 4% nickel and 1% manganese, of the manganese by, for example, 2.5% copper causes a much smaller loss of resistance to corrosion on the addition of sulphur. It is believed that the sulphur combines with the copper to form copper sulphide which is insoluble in dilute acids. Experiments have shown, and known data of free energy of formation of sulphides confirm, that, at the pouring temperature, the order of preferential combination with sulphur will be—manganese; copper; iron and chromium. Accordingly a steel containing copper to minimize the loss of resistance to corrosion must have the copper in a quantity exceeding that required to combine with the sulphur (i. e. a ratio exceeding 5:1) and must not contain substantial amounts of any metal, for example manganese or zirconium such as to combine with the sulphur in preference to copper.

A large excess of copper further assists the 45 machinability of the stainless steel.

In alloy steels formulated according to this

and C, a 10% solution of sulphuric acid at room temperature.

| No. | Constitution of Alloy |    |      |      |     | A     | B   | C      |
|-----|-----------------------|----|------|------|-----|-------|-----|--------|
|     | Cr                    | Ni | S    | Mn   | Cu  |       |     |        |
| 10  | 26                    | 4  | 0.01 | 0.9  | —   | 285   | 27  | 294    |
|     | 26                    | 4  | 0.3  | 0.9  | —   | 6,200 | 640 | 16,400 |
|     | 26                    | 4  | 0.3  | 0.01 | 2.5 | 178   | 7   | 10     |
|     | 26                    | 4  | 0.2  | 0.6  | 2.5 | 1,200 | 10  | 21,400 |
|     | 26                    | 4  | 0.3  | 0.01 | 5   | 4     | 11  | 48     |
|     | 26                    | 4  | 0.3  | 0.01 | —   | 400   | 5   | 3,680  |

It will be seen from the foregoing table that 15 the corrosion resistance of alloy No. 1 containing manganese is considerably reduced by the addition of sulphur as free cutting element (alloy No. 2). However, by the addition of copper and the virtual exclusion of manganese, alloy No. 3 20 is obtained which has better corrosion resistance to all treatments than alloys Nos. 1 or 2. This improved resistance is however substantially reduced by the reinclusion of manganese as shown by alloy No. 4. A further improvement is obtained in alloy No. 5 by the exclusion of manganese and the presence of a more substantial proportion of copper, and improved resistance in alloy No. 6 as compared with alloy No. 2 is obtained merely by the omission of the manganese, no copper being added.

Similarly improved resistance may be obtained 35 if the alloy contains molybdenum or vanadium. These elements form with sulphur, sulphides having a greater resistance to acid corrosion than iron sulphide and as they are formed preferentially at the pouring temperature they constitute further examples in accordance with the invention.

The following table shows the influence on 40 corrosion resistance of the addition of manganese to a sulphur bearing 18% chromium, 8% nickel, 2.5% molybdenum, cast stainless steel and it will be noted that on comparing alloys I and III, the advantages of free machining have been obtained without reduction of the corrosion resistance of steel I, such as is shown in the case of alloy II.

| Alloy Mark | Analysis    |             |             |             |            | Solution Rate                  |                        |                                         |
|------------|-------------|-------------|-------------|-------------|------------|--------------------------------|------------------------|-----------------------------------------|
|            | Cr, Percent | Ni, Percent | Mo, Percent | Mn, Percent | S, Percent | Boiling 1% Lactic Acid+1% salt | Boiling 1% Nitric Acid | 10% cold H <sub>2</sub> SO <sub>4</sub> |
| I          | 18.5        | 6.0         | 2.6         | 1.1         | 0.04       | 16                             | 1                      | 23                                      |
| II         | 18.1        | 7.8         | 2.5         | 1.1         | 0.34       | 118                            | 13                     | 63                                      |
| III        | 18.1        | 8.0         | 2.3         | 0.1         | 0.32       | 1                              | 1                      | Nil                                     |

invention and which do not contain copper, manganese or zirconium, the acid-insoluble separate phase responsible for the easy breaking of swarf may be a complex of chromium and iron sulphides such as  $Fe(CrS_2)_2$ , which is known to be substantially unaffected by dilute acids.

Alloy steels of the present invention contain 65 21% to 29% chromium, 4% to 6% nickel, 0.10% to 0.75% sulphur, and a manganese content not greater than 0.4%.

The following table shows the improvement in 70 results obtained with alloys formulated in accordance with the present invention. The figures given under A, B and C are respectively the loss in milligrammes per sq. decimeter per day for; A, an aqueous solution containing 1% lactic acid and 1% sodium chloride at boiling point, B, a 1% aqueous solution of nitric acid at boiling point,

It should be noted that in the case of alloys to 60 composition II, considerable variations in corrosion resistance are encountered. The figure given in the above table for alloy II in boiling lactic acid plus sodium chloride has on occasion been found to be as high as 780. One of the advantages to be gained by the elimination of manganese as far as is practicable is that the variation of corrosion resistance of a given composition is greatly reduced. Experimental work suggests that when the sulphur content is about 0.3% the manganese should not be greater than 0.4% but is preferably below 0.2%.

It follows from the foregoing description that 75 an improved corrosion resistance in steels containing chromium, nickel, molybdenum or vanadium, singly or together, and which contain sulphur as the free cutting element, is achieved by

the substantial exclusion of manganese or zirconium from the steels. In general the corrosion resistance of such steels, to which free cutting elements have been added to improve machinability, may be maintained by ensuring in the manner detailed, that the separate phase on which the free cutting depends is insoluble in dilute acids.

We claim:

1. Alloy steels consisting of iron alloyed with 21-29% chromium, 4-6% nickel, 0.10-0.75% sulphur and wherein the manganese content is not greater than 0.4% and preferably below 0.2%.
2. Alloy steels consisting of iron alloyed with 21-29% chromium, 4-6% nickel, 0.10-0.75% sulphur and a proportion of copper relative to sul-

phur of at least 5:1 and wherein the manganese content is not greater than 0.4%, preferably below 0.2%.

5 References Cited in the file of this patent

UNITED STATES PATENTS

| Number    | Name   | Date         |
|-----------|--------|--------------|
| 1,961,777 | Palmer | June 5, 1934 |

OTHER REFERENCES

Stainless Iron and Steel, Second and Revised Edition, pages 249 and 250, edited by Monyhenny, published in 1931 by Chapman and Hall, Limited, London, England.